

Nov. 1, 1927.

1,647,822

R. V. WILLIAMS

SPINNERETTE

Filed Oct. 12, 1925

Fig. 1.



Fig. 2.



Inventor,  
Reginald V. Williams,  
by Geiger & Geiger  
Attorneys.

Patented Nov. 1, 1927.

1,647,822

# UNITED STATES PATENT OFFICE.

REGINALD V. WILLIAMS, OF BUFFALO, NEW YORK.

## SPINNERETTE.

Application filed October 12, 1925. Serial No. 61,905.

This invention relates to the spinnerettes used in the manufacture of artificial silk or the so-called rayon products. These consist of metallic caps or nozzles mounted on rotary spindles and provided in their closed ends with perforations through which the usual chemical composition is forced for producing the artificial silk threads or filaments.

The object of my invention is the production of a spinnerette which can be produced at a comparatively low cost and which, while resisting the action of acid and alkaline solutions, has the required hardness and strength, and is sufficiently malleable to permit its easy stamping without danger of cracking or fracture.

To that end the invention consists in making the spinnerette of an alloy of gold and nickel.

20 In the accompanying drawings:—

Figure 1 is a side elevation of a spinnerette embodying the invention. Figure 2 is a longitudinal section thereof.

Similar characters of reference indicate 25 corresponding parts in both the views.

The spinnerette has the form of the usual cap or nozzle 10 having a base flange 11 and provided in its head with a plurality of perforations 12 for the passage of the chemical 30 composition or pulp which produces the artificial threads. The improved spinnerette is formed or stamped from an alloy composed

of pure gold or twenty-four karat gold and nickel, preferably in the proportion of eighty to ninety-nine percent of gold and one to 35 twenty percent of nickel. These metals are heated in a crucible or furnace to sufficiently high temperature to form a homogeneous alloy, after which the alloy is cast in a suitable mold and rolled into sheets which are 40 then stamped in appropriate dies to form the spinnerettes.

While being light, strong, hard and durable, these improved spinnerettes are unaffected by the acids or chemical solutions 45 used for producing the artificial silk or rayon products and they can be produced at considerably less cost than the spinnerettes heretofore used.

At the same time, the alloy of which the 50 spinnerettes are made, possesses the necessary malleability to permit them to be easily stamped.

I claim as my invention:—

1. A spinnerette constructed of an alloy 55 composed of gold and nickel.

2. A spinnerette constructed of an alloy composed predominantly of gold and a materially less percentage of nickel.

3. A spinnerette constructed of an alloy 60 composed of from eighty to ninety-nine percent of gold and from one to twenty percent of nickel.

REGINALD V. WILLIAMS.